

W. B. SULLIVAN,  
PERCUSSION TOOL.  
APPLICATION FILED MAY 11, 1918.

1,296,338.

Patented Mar. 4, 1919.



Inventor  
William B. Sullivan  
by  
Gillson & Gillson  
Attorneys

# UNITED STATES PATENT OFFICE.

WILLIAM B. SULLIVAN, OF CHICAGO, ILLINOIS.

## PERCUSSION-TOOL.

1,296,338.

Specification of Letters Patent.

Patented Mar. 4, 1919.

Application filed May 11, 1918. Serial No. 233,942.

To all whom it may concern:

Be it known that I, WILLIAM B. SULLIVAN, a citizen of the United States, and resident of Chicago, county of Cook, and State 5 of Illinois, have invented certain new and useful Improvements in Percussion-Tools, of which the following is a specification, and which are illustrated in the accompanying drawings, forming a part thereof.

10 The invention relates to punches, rivet sets and the like, and especially to those tools which are operated by being driven with great force against the work and which may be repeatedly heated and cooled in service as 15 by intermittent use upon a heated objective. The object of the invention is to provide a tool of great efficiency and durability for use either upon hot or cold work, and of such a character that skilful heat treatment 20 is not required for obtaining the most desirable condition of the tool, as to hardness.

The single figure of the accompanying drawing shows a rivet set designed for use with so-called air hammers and which it is 25 proposed should embody the present invention, a part of the tool being shown in section.

The service to which tools, as 10, are subjected makes it desirable that they should 30 have the required degree and character of hardness to perform the operations for which they are intended and at the same time afford great resistance against wear, either by abrasion or distortion, particularly 35 at the head 11 and shank 12. In order that the tool may be used upon both heated and cold objectives it is also required that it should have great longitudinal and transverse strength in the required hardness state 40 and that all of these properties should be retained at the highest temperatures which may be attained in any part of the tool in service, as also after subsequent cooling. That is to say, the tool should have high 45 red hardness and be free from air hardening properties. Abrasion or distortion of the tool when the head, as 11, is driven against a heated objective and brittleness due to excessive hardness, after repeated use, are 50 thus avoided. The strength and hardness required for cold operations is thereby retained even after long continued service.

It is accordingly proposed that the improved tool, as 10, should have a fixed metalloptic structure to a high temperature and 55 should be capable of being quenched in

either oil or water from any higher temperature throughout a wide range without producing excessive hardness. For this purpose the invention contemplates a tool 60 formed from steel comprising an unusually high proportion of silicon. It has been found that remarkable results are obtained with tools formed from steel having the following composition:—

|           |               |
|-----------|---------------|
| Silicon   | 1.75 to 2.25% |
| Manganese | .50 to 1.00%  |
| Carbon    | .50 to .65%   |

Such a tool may be made from open 70 hearth steel and it will be of substantially the same hardness if quenched in either oil or water from any temperature between 1500° and 1900° F.

The relatively large proportion of silicon 75 is believed to render the metalloptic state or condition of the tool obtained by quenching, stable to any temperature likely to be attained in any part of the tool in use upon hot work without imparting the air hardening properties which would cause the tool to become excessively hard and brittle in service. Furthermore, the wide range of temperatures from which the tool may be quenched with substantially uniform results 80 renders skilful treatment unnecessary while the hardness and strength are sufficient to permit long continued use in any punching operation without fracture or change of size or form beyond the usual limits of tolerance. 85 The invention accordingly provides an inexpensive tool of the required hardness and strength for any piercing or punching operation upon either hot or cold work and most extraordinary results with respect to durability of the tool in long continued service. 90 95

While reheating the tool, as 10, after quenching to any temperature which does not closely approximate 900° F. does not 100 materially change its hardness, for the purpose of relieving internal strains it may be desirable to bring the tool to a uniform temperature of about 600° F., after quenching, particularly if the tool is of irregular shape, as shown. It will be understood that the essential hardness required for the particular class of tools indicated is determined by their composition. That is to say, substantially the same hardness is obtained by quenching from any temperature above 1500° F. through a wide range, and this 105 110

hardness is not modified by reheating to lower temperatures. The improved tool is thus distinguished from tools of so-called straight carbon steel wherein the hardness obtained is determined by the temperature to which the tool is reheated after quenching.

The improved tool is also distinguished from tools of any of the alloy steels by being free from air hardening properties. These distinctions are believed to be due to differences in the character of the martensite produced by quenching the different tools from temperatures above the decalescent points of the corresponding steels. That of the so-called straight carbon steel tools is hard and brittle but rapidly decomposes when the tool is reheated after quenching. On the other hand, that of the alloy steels is originally hard and strong, retains its hardness and strength to high temperatures but increases in hardness and becomes brittle upon subsequent cooling in the air. The martensite produced by quenching the tool provided by the present invention differs from both in being stable up to temperatures at which the hardness obtained in so-called straight carbon steels by quenching would be substantially destroyed and air-hardening steels would be materially modified. The tool is described in the accompanying claims as comprising an impact-receiving shank and a punch head with a view to indicating that it is specially formed for engagement with the objective and to provide a place where it may be struck to afford the impulse by which the work is performed, but this expression is not intended to indicate that the head and shank are necessarily of different dimensions, as shown.

I claim as my invention—

1. A percussion tool for punching, rivet setting, and like hot or cold operations, comprising an impact receiving shank and a

punch head composed of steel containing approximately two per cent. silicon.

2. A percussion tool for punching, rivet setting, and like hot or cold operations, comprising an impact receiving shank and a 50 punch head composed of steel containing approximately two per cent. silicon, manganese in appreciable quantity not substantially exceeding one per cent., and approximately one-half per cent. carbon.

3. A percussion tool for punching, rivet setting, and like hot or cold operations, comprising an impact receiving shank and a punch head composed of steel containing one and three-quarters to two and one-quarter per cent. silicon, one-half to one per cent. manganese, and one-half to sixty-five one-hundredths per cent. carbon. 55 60

4. A percussion tool for punching, rivet setting, and like hot or cold operations, comprising an impact receiving shank and a punch head composed of steel containing iron as its principal ingredient and silicon largely in excess of any ingredient other than iron, the amount of the silicon content 65 70 being approximately two per cent.

5. A percussion tool for punching, rivet setting, and like hot or cold operations, comprising an impact receiving shank and a punch head composed of steel consisting of iron as its principal ingredient combined with another substance having the property of silicon in imparting to the steel, when approximately two per cent. is used therein, the quality of red hardness without air-hardening properties. 75 80

6. A percussion tool for punching, rivet setting, and like hot or cold operations, comprising an impact receiving shank and a punch head composed of steel having, after 85 quenching, the red hardness characteristic of self-hardening steels without the property of air hardening.

WILLIAM B. SULLIVAN.